

# UNITED STATES PATENT OFFICE.

GEORG HEBERLEIN, OF WATTWIL, SWITZERLAND.

## PROCESS FOR PRODUCING WOOL-LIKE EFFECTS ON COTTON FABRICS.

1,288,884.

Specification of Letters Patent. Patented Dec. 24, 1918.

No Drawing.

Application filed May 18, 1916. Serial No. 98,295.

To all whom it may concern:

Be it known that I, Dr. GEORG HEBERLEIN, a citizen of the Swiss Republic, and resident of Wattwil, canton of St. Gall, Switzerland, have invented a new and useful Process for Producing Wool-Like Effects on Cotton Fabrics, of which the following is a full, clear, and exact specification.

If a mercerized fabric be treated with a 10 sulfuric acid of about 49 to 50 $\frac{1}{2}$ ° Baumé, a particular wool-like effect is produced as is described in my U. S. Letters Patent No. 1141872 dated June 1, 1915. Similar changes in the cotton take place if the fabric be 15 first treated with sulfuric acid of 49 to 50 $\frac{1}{2}$ ° Baumé and then acted upon with concentrated soda-lye.

From the foregoing statement it is obvious that on the one hand the action of the 20 sulfuric acid is the more intense if the cotton has been previously treated with soda-lye and on the other hand that a cotton which has been subjected to the action of concentrated sulfuric acid comports itself 25 differently during the subsequent treatment with soda-lye than is the case with cotton which has not been thus previously treated.

I have now found that still more extensive modifications of the cellulose and consequently increased woollike effects on cotton fabrics can be obtained by causing concentrated sulfuric acid of 49 to 50 $\frac{1}{2}$ ° Baumé and concentrated soda lye to act upon the 30 said fabrics several times alternately the sulfuric acid being always allowed to act each time for some minutes. If cotton, treated with concentrated soda-lye, is subjected for a second time to the same treatment no further alteration thereof takes place, that is to 35 say, the second treatment with soda-lye is without effect. Cotton behaves in an analogous manner in respect of the repeated action of concentrated sulfuric acid. If, however, the mercerized cotton is subsequently 40 subjected to the action of concentrated sulfuric acid then the soda-lye again reacts and effects a further change. The conditions are exactly the same if the first treatment is with concentrated sulfuric acid. If, in this 45 case, a treatment with soda-lye then follows, the concentrated sulfuric acid will again subsequently react. The alternate treatment with acid and alkali can be repeated several times, the number of manipulations natu-

rally being limited by the progressing solution of the cellulose. 55

In order to obtain increased woollike effects it is necessary that one or other of the two reagents shall be employed at least twice with the intermediate action of the other 60 agent, for example, soda-lye—sulfuric acid—soda-lye—or sulfuric acid—soda-lye—sulfuric acid. In between the reactions the goods must be well washed and if desired, subsequently dried. 65

It will be obvious that most varied woollike effects are to be obtained according to the number of manipulations and, moreover, according as to whether the first or last treatment takes place with concentrated 70 alkali lye or concentrated acid, the concentration of the sulfuric acid employed being always 49 to 50 $\frac{1}{2}$ ° Baumé as described in my already specified U. S. Letters Patent No. 1141872. Variations in the quality of the 75 fabric can also be obtained by more or less stretching the same in the longitudinal and transverse direction during one treatment or during several treatments that is to say by allowing it to shrink more or less. 80

Finally, pattern effects may be obtained by printing the acid or alkali at one or more of the operations only upon particular portions of the fabric, or by printing on particular portions of the fabric a resist (for instance gum thickening), either at the commencement of the operation or between the first and the second or between two successive operations, the said resist preventing a further reaction of the acid or alkali. Those 90 portions which are not printed with acid or alkali or which have been reserved show the fabric in its original or partly altered condition and differentiate themselves from the printed or un-reserved portions which have, 95 experienced a more thorough modification so that more or less sharp patterns are produced. 85

What I claim is:

1. The herein described process for imparting to cotton fabrics a wool-like appearance, consisting in causing concentrated alkali lye and sulfuric acid of 49 to 50 $\frac{1}{2}$ ° Baumé to act alternately and repeatedly upon the fabrics in such a manner that a 100 treatment with one of the said reagents takes place between two treatments with the other, the sulfuric acid being allowed to act on the 105

fabrics each time for some minutes, the fabrics being washed out after each treatment.

2. The herein described process for imparting to cotton a wool like appearance, consisting in causing concentrated alkali lye and sulfuric acid of 49 to 50 $\frac{1}{2}$ ° Baumé to act alternately and repeatedly upon the fabrics in such a manner that a treatment with one of the said reagents takes place between two 10 treatments with the other, the fabrics being stretched at least during one of the said treatments, the sulfuric acid being allowed to act on the fabrics each time for some minutes and the fabrics being washed out 15 after each treatment.

3. The herein described process for producing wool like pattern effects on cotton fabrics, consisting in causing concentrated alkali lye and sulfuric acid of 49 to 50 $\frac{1}{2}$ ° 20 Baumé to act alternately and repeatedly upon the fabrics in such a manner that a treatment with one of the said reagents takes place between two treatments with the other, at least at one of the said treatments the reagent employed being caused to react 25 only upon particular portions of the fabrics,

the sulfuric acid being allowed to act on the fabrics each time for some minutes and the fabrics being washed after each treatment.

4. The herein described process for producing wool-like pattern effects on cotton fabrics, consisting in causing concentrated alkali lye and sulfuric acid of 49 to 50 $\frac{1}{2}$  Baumé to act alternately and repeatedly 30 upon the fabrics in such a manner that a treatment with one of the said reagents takes place between two treatments with the other, the fabrics being stretched at least during one of the said treatments and at least at 35 one of the said treatments the reagent used being caused to react only upon particular portions of the fabrics, the sulfuric acid being allowed to act on the fabrics each time for some minutes and the fabrics being washed out 40 after each treatment.

In witness whereof I have hereunto signed my name this 29th day of April 1916, in the presence of two subscribing witnesses.

Dr. GEORG HEBERLEIN.

Witnesses:

F. BAUMRATZ,  
A. MATTES.